

# United States Patent Office

2,773,038

Patented Dec. 4, 1956

1

2,773,038

## LUBRICANTS

William B. Whitney and William N. Axe, Bartlesville, Okla., assignors to Phillips Petroleum Company, a corporation of Delaware

No Drawing. Application November 20, 1951,  
Serial No. 257,410

18 Claims. (Cl. 252—48.8)

This invention relates to new and improved lubricants. In one aspect this invention relates to improved lubricating oils containing selected sulfurized compounds as addition agents. In another aspect this invention relates to the preparation of materials having particularly utility as mineral lubricating oil addition agents.

At the present time it is common practice to enhance or modify certain of the properties of lubricating oils through the use of additives or improvement agents, to render the oil serviceable over the adverse conditions encountered, when employed in internal combustion engines such as automotive, aircraft, and diesel engines. Our invention is concerned with new lubricating oil additives or improvement agents, which when incorporated with a mineral oil employed as a lubricant in an engine of the internal combustion type, impart valuable improvements to the oil, particularly as regards corrosion inhibiting properties, and increased resistance of the oil to oxidation.

An object of this invention is to provide new lubricating oil compositions. Another object is to provide new mineral oil addition agents. Another object is to provide for an increase in the anticorrosion and antioxydation characteristics of a mineral lubricating oil. Another object is to provide a class of mineral lubricating oil addition agents, which when incorporated with a mineral lubricating oil in service in an internal combustion engine of the type above described, greatly reduce the corrosive action of the oil on engine bearing parts, and increase its resistance to oxidation. Other objects will be apparent to those skilled in the art in the light of the accompanying disclosure.

In accordance with our invention we provide as new lubricant compositions, a mineral lubricating oil containing in solution a minor proportion of a sulfurized diarylalkane. Our invention is based on our discovery that diarylalkanes can be sulfurized to form a product material, which when dissolved in a mineral lubricating oil improves the resistance of the oil to oxidation and inhibits corrosive action of the oil on engine parts in contact therewith.

The sulfurized diarylalkane addition agents of our invention are those produced by sulfurization of diarylalkanes, when employing sulfur monochloride as the sulfurizing agent either non-catalytically or in the presence of a catalyst, as described hereinafter. Diarylalkanes to be sulfurized to produce our addition agents contain the two aryl groups preferably attached to alkane carbon atoms either adjacent each other or separated by no more than one carbon atom. The aryl groups of the diarylalkane can be the same or different and are comprised of phenyl, naphthyl, anthryl and phenanthryl radicals, substituted or unsubstituted.

The diarylalkane to be sulfurized can be produced in any desired manner. One preferred method involves the alkylation of an aromatic compound such as benzene, naphthalene, anthracene, phenanthracene, or such aro-

2

matics substituted, as for example toluene, xylene, phenol, dimethyl naphthalene, diethyl naphthalene, diethyl naphthalene, di-tert-butyl anthracene, di-isoamyl-phenanthrene, tri-tert-butyl phenanthrene, methyl-tert-butyl naphthalene, ethylidodecyl benzene, cumene, and the like, and particularly long-chain alkyl aromatics, with conjugated diolefins often containing from 4 to 6 carbon atoms, as for example, 1,3-butadiene, 1,3-pentadiene, 1,3-hexadiene, 2-methyl-1,3-pentadiene, and the like. Other diolefins particularly representative of those that can be alkylated with an aromatic to produce the diarylalkane to be sulfurized include, conjugated dodecadiolefins, viz. 1,3-, 2,4-, 3,5-, 4,6- and 5,7-conjugated octadienes, conjugated heptadienes, or such dienes alkyl substituted. Such an alkylation can be effected under any appropriate alkylating conditions and in the presence of a suitable catalyst as, for example, hydrogen fluoride, boron fluoride, a boron trifluoride-water complex, a complex of boron trifluoride with aqueous hydrogen fluoride, aluminum chloride, and the like, the specific alkylating temperature and time conditions being characteristic of those generally employed in conjunction with the particular alkylation catalyst employed.

The sulfurization of the diarylalkane is conducted, employing sulfur monochloride as the sulfurizing agent, generally at a temperature within the limits of 20 and 110° C., and preferably within the narrow range of about 40 and 60° C. However, the rate of sulfurization reaction varies considerably depending on the particular substituents on the aryl radical, if any and on their position. For example, those diphenylalkanes in which the para position of the phenyl group is occupied, sulfurize much more slowly than when the para position is free. In such a case, i. e. when the para position is substituted, a higher temperature is generally preferred, the optimum level likely being between about 60 and 110° C., so as to effect the desired sulfurization in a reasonable length of time. However, the rate of the sulfurization can be increased also by effecting the reaction in the presence of a suitable catalyst, such as zinc dust. Accordingly, if desired, we can increase the rate of the sulfurization by increasing the sulfurization temperature, or by the use of a suitable catalyst, or both. If time is too short, conversion is low; if too high, some of the desired oil soluble product is converted into insoluble material. The optimum reaction time will depend on other reaction variables such as the mol ratio of sulfur monochloride to the diarylalkane, presence and character of a catalyst, temperature and the like. The optimum time may be determined by routine test. For the sulfurization conditions illustrated in the examples, a sulfurization time of from 30 to 100 minutes is preferable.

The addition agent of our invention appears to be formed by coupling of sulfurized monomers and non-sulfurized monomers (the selected diarylalkane) together with sulfur to form the resulting sulfur-containing "polymer." In carrying out the sulfurization it is important to effect the careful control of the sulfurization conditions to form highest yields of oil-soluble sulfur containing product. Accordingly it is important to effect the sulfurization within the reaction time above described, by carefully selecting the requisite temperature level, and if needed, a suitable catalyst, as well as to employ a mol ratio of sulfur monochloride to the diarylalkane, introduced into the sulfurization zone within the preferred range which we have found to be about 0.5:1 to 2.0:1. The sulfurization product portions soluble in benzene, or in benzene-pentane mixture generally containing at least 80 volume percent benzene, exhibit good solubility in the lubricating oil and are preferred addition agents of our invention.

Any desired mineral oil base having lubricating properties, and of suitable grade and viscosity can be employed in compounding our improved lubricating oil compositions. Exemplary of our preferred base materials are mineral oils having a viscosity at 100° F. as low as 45 SUS and as high as 100 SUS at 210° F.; and a viscosity index at least as high as 50. In compounding our compositions we generally add from 0.1 to 10 percent by weight of the addition agent to the lubricating oil base (based on the weight of the resulting composition), although more often we find that from 0.3 to 3.0 weight percent of the addition agent is sufficient. The amount of addition agent employed will be determined to an extent by the characteristics of the selected oil base, and also upon the service conditions to which the compositions are to be subjected. Although the concentration of addition agent employed will not generally exceed 10 percent, higher concentrations can be employed, if desired.

The addition agents of our invention function independently of other types of additives without materially altering the physical characteristics of the oil, and accordingly, the base oil may contain other additive agents, such as viscosity index improvement agents, pour point depressants, and the like.

Our invention is illustrated by the following examples. The reactants, their proportions, and other specific ingredients are presented as being typical and should not be construed to limit the invention unduly.

*Example 1*

Xylene, introduced into an alkylation zone with 1,3-butadiene in a mol ratio to butadiene of approximately 10:1 (3.7 pounds of total reactants), was alkylated with the butadiene at atmospheric pressure and at a temperature of 60 to 70° F. in the presence of a  $\text{BF}_3\text{-HF-H}_2\text{O}$  catalyst, to form dixylylbutane. The catalyst was prepared by saturating 47 percent aqueous HF with  $\text{BF}_3$ . The catalyst volume was 10 percent of the total volume of catalyst and reactants. The alkylation was a batch reaction, and the purified product had a boiling range of 624 to 660° F. (atmospheric pressure) and a specific gravity at

60° F.

60° F.

of 0.9606.

1.50 moles of sulfur monochloride was added to 1.18 moles of the purified dixylylbutane, together with approximately 40 grams of zinc dust, employing 300 cc. benzene as a diluent. Previous experiments showed that no reaction took place with benzene and sulfur monochloride in presence of zinc, below a temperature of 70° C. The resulting admixture was warmed to 45° C., thus starting the reaction, and was then cooled to 25 to 30° C. where most of the reaction was permitted to take place. Toward the end of the reaction the temperature was raised to 40° C. The reaction admixture contained an excess of sulfur monochloride, a major proportion of which was separated from the sulfurized product, together with the benzene diluent by vacuum distillation, at the end of the reaction period. The sulfurized product was treated with isopropyl alcohol to decompose the remaining sulfur monochloride. The sulfurized dixylylbutane was further purified by extraction in a benzene-pentane solution. In carrying out the extraction, 100 grams of the sulfurized dixylylbutane was dissolved in an equal volume of pentane and charged to a silica gel column already wet with pentane. The column was washed thoroughly with pentane to remove the sulfur. In copending application Serial Number 250,565, filed October 9, 1951, there are described and claimed processes for the removal of elementary sulfur from its admixture with a sulfurized hydrocarbon compound employing silica gel. Upon washing with 20 percent benzene in pentane, the sulfurized dixylylbutane was obtained

from the silica gel. This material diluted with toluene was boiled with barium oxide for three hours. Xylene was added to distill out the residual toluene and then the xylene was distilled. The product was stripped with gas up to 180° C. The purified sulfurized dixylylbutane was found upon analysis to contain 12.03 weight percent sulfur, 0.10 weight percent ash and 1.37 weight percent chlorine, and was tested as described in Example 3.

*Example 2*

Toluene was introduced into an alkylation zone, with 1,3-butadiene in a mol ratio to butadiene of approximately 10:1 (2.65 pounds of total reactants) and alkylated with the butadiene at atmospheric pressure and at a temperature of 65 to 75° F. in the presence of a  $\text{BF}_3\text{-H}_2\text{O}$  catalyst, to form ditolylbutane. The catalyst was prepared by making a saturated solution of  $\text{BF}_3$  in water. The catalyst volume was 10 per cent of the total volume of catalyst and reactants. The alkylation was a batch reaction, 167 minutes in duration. The ditolylbutane product was purified by distillation. The purified product had a boiling range of 606 to 608° F., at atmospheric temperature and a specific gravity at

60° F.

60° F.

of 0.9626.

1.25 moles of sulfur monochloride was added to 1.25 moles of the purified ditolylbutane together with about 35 grams of zinc dust, again employing benzene as a diluent. The reaction temperature was maintained 50 to 55° C. for about one hour. The temperature toward the end of the reaction was raised to 70° C. The reaction admixture contained an excess of sulfur monochloride, a major proportion of which, together with the benzene diluent was separated from the sulfurized product, by vacuum distillation. The sulfurized product was treated with isopropyl alcohol to decompose the remaining sulfur monochloride. The purified sulfurized product was then tested as described in Example 3.

*Example 3*

The following lubricating oil compositions were prepared from the lubricating oil base stock described herebelow, and the sulfurized dixylylbutane and sulfurized ditolylbutane products described in the preceding examples.

The oil employed as the base oil in these compositions was a solvent-refined Mid-Continent oil of lubricating grade having the following characteristics:

|                               |      |
|-------------------------------|------|
| Gravity API                   | 30.4 |
| Viscosity at 210° F. S. U. S. | 58.5 |
| Viscosity index               | 97   |
| Neutralization                | 0.01 |

| Composition                                           | I     | II   | III  | IV   | V    |
|-------------------------------------------------------|-------|------|------|------|------|
| Base-Lubricating Oil, Weight Percent                  | 100.0 | 99.5 | 99.0 | 99.5 | 99.0 |
| Sulfurized dixylylbutane, <sup>1</sup> Wt. Percent    | 0.0   | 0.5  | 1.0  | 0.0  | 0.0  |
| Sulfurized ditolylbutane, <sup>2</sup> Weight Percent | 0.0   | 0.0  | 0.0  | 0.5  | 1.0  |

<sup>1</sup>Purified product of Example 1.

<sup>2</sup>Purified product of Example 2.

These compositions were evaluated in a mounted single cylinder H-2 Lauson test engine. The test performed consisted in placing 900 grams of the composition in the crankcase of the single cylinder Lauson (gasoline) engine, and operating the engine under a 1.2 H. P. load at 1600±20 R. P. M., while maintaining a cooling jacket temperature of 210° F., an oil temperature of 310° F. and an air-to-fuel ratio of 13.5:1. At the end of 60 hours' operation under these conditions the test engine was stopped, disassembled and examined.

The bearing weight loss, in milligrams, encountered in each test was as follows:

| Lubricating Oil Tested              | Percent Additive in Oil | Bearing Weight Loss, Mg. |
|-------------------------------------|-------------------------|--------------------------|
| Base Oil                            | 0                       | 870.8                    |
| Base Oil + Sulfurized Dicylbutane   | 0.5                     | 48.8                     |
| Do                                  | 1.0                     | 16.0                     |
| Base Oil + Sulfurized ditolylbutane | 0.5                     | 49.0                     |
| Do                                  | 1.0                     | 14.0                     |

It will be seen from these data that the addition of a relatively small proportion of an improvement agent of our invention, to a typical crankcase lubricant, decreases the bearing weight loss to a satisfactory low value.

While the invention has been described in connection with a present, preferred embodiment thereof, it is to be understood that this description is illustrative only and is not intended to limit the invention.

We claim:

1. As a new composition, a mineral lubricating oil containing an amount sufficient to impart anticorrosion properties thereto, of a product of sulfurization of a diarylalkane containing from 4 to 12 alkane carbon atoms obtained when employing sulfur monochloride as the sulfurizing agent.

2. A lubricating oil composition comprising a mineral oil having a viscosity index of at least 50 and containing an amount sufficient to impart anticorrosion properties thereto, of a product of sulfurization of a diarylalkane containing from 4 to 12 alkane carbon atoms, obtained when employing sulfur monochloride as the sulfurizing agent.

3. The composition of claim 2 wherein said diarylalkane is a diphenyl alkane.

4. The composition of claim 3 wherein said diphenylalkane is dixylbutane.

5. The composition of claim 3 wherein said diphenylalkane is ditolylbutane.

6. A lubricating oil composition comprising a mineral lubricating oil containing from 0.1 to 10 percent by weight, based on said composition, of a product of sulfurization of a diarylalkane containing from 4 to 12 alkane carbon atoms obtained when employing sulfur monochloride as the sulfurizing agent.

7. The composition of claim 6 containing from 0.1 to 3 weight percent of said sulfurized diarylbutane.

8. A lubricating oil composition comprising a mineral lubricating oil containing from 0.1 to 10 weight percent of a product of sulfurization of diphenylbutane obtained when employing sulfur monochloride as the sulfurization agent.

9. A lubricating oil composition comprising a mineral lubricating oil containing from 0.1 to 10 weight percent of a product of sulfurization of ditolylbutane obtained when employing sulfur monochloride as the sulfurization agent.

10. As a new composition, a mineral lubricating oil containing an amount sufficient to impart anticorrosion properties thereto, of a product of sulfurization of a diarylalkane containing from 4 to 12 alkane carbon atoms

obtained when employing sulfur monochloride as the sulfurizing agent.

11. As a new composition, a mineral lubricating oil containing an amount sufficient to impart anticorrosion properties thereto of a product of sulfurization of a diarylalkane, obtained when employing sulfur monochloride as the sulfurizing agent, said diarylalkane having been prepared by the alkylation of an aromatic hydrocarbon with a conjugated diolefin hydrocarbon containing from 4 to 12 carbon atoms in the molecule, and said sulfurization having been conducted at a temperature in the range of 20-110° C.

12. The composition of claim 11 wherein said diolefin hydrocarbon reactant contains from 4 to 6 carbon atoms in the molecule.

13. A composition of claim 12 wherein said diolefin is 1,3-butadiene and said aromatic hydrocarbon is xylene.

14. A composition of claim 12 wherein said diolefin is 1,3-butadiene and said aromatic hydrocarbon is toluene.

15. As a new composition, a mineral lubricating oil containing an amount sufficient to impart anticorrosion properties thereto of a product of sulfurization of a diarylalkane, obtained when employing sulfur monochloride as the sulfurizing agent, said diarylalkane having been prepared by the alkylation of an aromatic hydrocarbon with a conjugated diolefin hydrocarbon containing from 4 to 12 carbon atoms in the molecule, and said sulfurization having been conducted at a temperature in the range of 20-110° C. with sulfur monochloride having been introduced into the sulfurization zone in a mol ratio to said diarylalkane therein in the range of from about 0.5:1 to 2:1, and for a period of from 30 to 100 minutes.

16. A composition of claim 15 wherein said aromatic hydrocarbon is selected from the group consisting of benzene, naphthalene, anthracene, phenanthrene, toluene, xylene, phenol, dimethyl naphthalene, diamyl naphthalene, diethyl naphthalene, di-tert-butyl anthracene, di-isoamyl phenanthrene, tri-tert-butyl phenanthrene, methyl-tert-butyl naphthalene, ethylidodecyl benzene and cumene, and wherein said diolefin is selected from the group consisting of 1,3-butadiene, 1,3-pentadiene, 1,3-hexadiene, 2-methyl-1,3-pentadiene, 1,3-dodecadiene, 2,4-dodecadiene, 3,5-dodecadiene, 4,6-dodecadiene, 5,7-dodecadiene, conjugated heptadiene and conjugated octadiene.

17. A composition of claim 15 wherein said sulfurization is effected in presence of zinc as a catalyst.

18. A composition of claim 2 wherein said diarylalkane contains said aryl groups attached to alkane carbon atoms, which atoms are separated by no more than one carbon atom.

#### References Cited in the file of this patent

#### UNITED STATES PATENTS

|           |                 |               |
|-----------|-----------------|---------------|
| 2,176,632 | Magill          | Oct. 17, 1939 |
| 2,244,886 | Lincoln et al.  | June 10, 1941 |
| 2,253,228 | Cantrell et al. | Aug. 19, 1941 |
| 2,380,072 | Reid            | July 10, 1945 |
| 2,429,691 | Johnson et al.  | Oct. 28, 1947 |
| 2,439,228 | Sturrock et al. | Apr. 6, 1948  |
| 2,497,138 | Rogers          | Feb. 14, 1950 |